

Aug. 31, 1926.

C. P. BYRNES

1,597,953

MANUFACTURE OF SHEET AND WIRE GLASS.

Original Filed June 19, 1920 2 Sheets-Sheet 2

Fig. 3.



Fig. 4.



Inventor

C. P. Byrnes

Aug. 31, 1926.

1,597,953

C. P. BYRNES

MANUFACTURE OF SHEET AND WIRE GLASS

Original Filed June 19, 1920 2 Sheets-Sheet 1

*Fig. 1.*



*Fig. 2.*



*Inventor*

*C. P. Byrnes*



Patented Aug. 31, 1926.

1,597,953

# UNITED STATES PATENT OFFICE.

CLARENCE P. BYRNES, OF SEWICKLEY, PENNSYLVANIA.

## MANUFACTURE OF SHEET AND WIRE GLASS.

Application filed June 19, 1920, Serial No. 390,116. Renewed June 27, 1925

Figure 1 is a diagrammatic vertical section showing one form of apparatus for carrying out my invention;

Figures 2, 3 and 4 are similar views showing other forms of apparatus.

My invention has relation to the manufacture of sheet glass, preferably in the form of wire glass, and particularly to the drawing of a plurality of sheets in a general vertical direction, and then bending the same in a general horizontal direction, embedding the wire mesh between the sheets while they are being drawn.

In the drawings, referring to the form of Figure 1, 2 represents the hearth or end portion of a glass tank furnace in which the molten glass is maintained at substantially the same level. This may be kept heated in any desirable manner. 3 is a horizontal bending roll which preferably has above it coacting roll 4, to press the sheets together with a mesh between. These rolls may be positively driven and may be intergeared or not, as desired. 5, 5 are sets of edge rolls engaging the edges of the sheets as they are drawn to retain their width. These rolls may either be positively driven or may be idle rolls with friction brakes which are adjustable to regulate the amount of drag imparted to the sheets. 6, 6 designate water-cooling devices extending across the bath at each side of the rising sheet. 7 indicates a roll of wire mesh which in this form is drawn between the right hand pair of edge rolls 5, thus becoming united with the under surface of the right hand sheet. The sheet with the wire mesh attached then passes up between the bending rolls 3 and 4, where it joins another sheet, both being united between the bending roll and the presser roll above it. 8 represents a heating burner in the form of a pipe extending between the sheets adjacent to the bending roll and reheating the adjoining faces of the sheets, in order to provide more effective embedding of the wire mesh. 9, 9 are fire-polishing burners adapted to fire polish the top and bottom surfaces of the wire glass. 10 indicates any desirable form of flattening and pulling devices by which the mesh is passed on through the leer, the end of which may be cut into any desirable sizes.

In the operation, the sheets are drawn up continuously, the wire mesh continuously feeds between the right hand pair of edge

rolls, and the three layers are joined at the bending joint, the wire mesh becoming embedded at the center of the wire glass thus formed.

In Figure 2, the roll of wire mesh 7<sup>a</sup> is beneath the hearth 2 and passes up through a slotted nozzle 11 extending upwardly through the hearth. It thence passes over a water-cooled roll 12, through the edging rolls 5<sup>a</sup>, where it joins the right hand sheet. The coolers 6<sup>a</sup> are here shown as water-cooled rollers, although any or all of them may be rotated, or not, as desired. In this case, the burners 8<sup>a</sup> and 9<sup>a</sup> are shown as in Figure 1, and the general operation is the same as in the first form.

In Figure 3, I show a form similar to Figure 1, except that the wire mesh 7<sup>b</sup> is placed between the sheets and the mesh is led directly to the bending roll, thus becoming embedded between the two sheets at the same time. Parts similar to Figure 1 are marked with similar numerals with the letter "b" applied. In this case, the burners 8<sup>b</sup> are shown in multiple to reheat the adjacent surfaces of the sheets before the wire mesh engages therewith at the bending roll.

In Figure 4, I show another form, generally similar to Figure 2, except that the wire mesh passes directly over a water-cooled roller 6<sup>c</sup> to the juncture of the sheets at the bending roll. In this case, parts similar to those of previous figures are marked with the same numeral with the letter "c" applied.

The advantages of my invention result from the cheap, simple and effective method provided for drawing sheet glass and for continuously drawing wire glass by forming a plurality of sheets, bending them in a horizontal direction, and simultaneously embedding the wire mesh therein. Wire glass may thus be cheaply and expeditiously made. Certain features of the invention are also applicable to and of advantage in drawing sheet glass.

The wire mesh fabric may be wider than or of the same width or narrower than the sheets of glass being drawn, and is preferably wider, so that portions of the wire mesh project beyond the edges of the sheet. The wire mesh may be partially cut across through intermediate portions at spaced intervals where the glass is to be cut at the exit of the leer, to facilitate cut-

ting of the sheets as the continuous feed progresses. The edge rolls 5 may extend across the sheet, the bending roll and its coacting presser roll may be employed to draw the sheets, and other variations may be made, without departing from my invention.

I claim:

1. In the manufacture of wire glass, the steps consisting of drawing a layer portion of glass upwardly from a molten bath, drawing another layer portion upwardly separate from the first layer portion, deflecting one layer portion, prior to uniting it with the other, feeding wire mesh between the glass layers, uniting the layers, and drawing the wire glass in a horizontal direction in a continuous manner.
2. In the manufacture of glass, the steps consisting of drawing a layer portion of glass upwardly from molten bath, drawing upwardly another layer portion of glass separate from the first named portion, deflecting one layer portion separately from the other, and then bringing the layers into contact, and drawing them in a generally horizontal direction in a continuous manner.
3. In the manufacture of wire glass, the steps consisting of continuously directing a plurality of sheets upwardly in a general vertical direction from a bath of glass, bending the sheets into another direction at the place where one of said sheets first changes its general vertical direction, and continuously embedding the wire mesh between the sheets at said place, substantially as described.
4. In the manufacture of wire glass, the steps consisting of drawing a plurality of sheets in a general vertical direction, reheating the adjacent surfaces of the sheets, embedding wire mesh between them, and bending the combined layers over a bending device, substantially as described.
5. In the manufacture of wire glass, the steps consisting of drawing a plurality of sheets in a general vertical direction, reheating the adjacent surfaces of the sheets, embedding wire mesh between them, bending the combined layers over a bending device, and fire polishing the surface of the wire glass as it is formed, substantially as described.
6. In the manufacture of wire glass, the method which consists in drawing a plurality of sheets upwardly in a general vertical direction from a bath of glass, unrolling a roll of wire mesh at a level above the bath, and embedding said wire mesh between said sheets, substantially as described.
7. In the manufacture of wire glass, the method consisting in drawing a plurality of sheets upwardly in a general vertical direction from a bath of molten glass, bending them into a different direction, unrolling a

roll of wire mesh at a level above the bath and feeding the wire mesh between the sheets, substantially as described.

8. In the manufacture of wire glass, the steps consisting of drawing a layer portion of glass upwardly from a molten bath, drawing upwardly another layer portion of glass separately from the first named portion, feeding wire mesh between the glass layer portions, changing the direction of travel of the wire mesh prior to uniting the layers and the mesh, and thereafter uniting the three layers.

9. In the manufacture of wire glass, the steps consisting of drawing a layer portion of glass upwardly from the molten bath, drawing upwardly another layer portion of glass separately from the first named portion, feeding wire mesh into contact with the inner face of one glass layer, and thereafter uniting the three layers and carrying them in a generally horizontal direction.

10. In the manufacture of sheet glass, the steps consisting of drawing a sheet vertically from a bath of molten glass, acting upon the outer portions of the rising sheet with edge rollers while leaving its intermediate portion free, and deflecting the sheet into another path at an angle to the vertical and horizontal after it passes the edge rollers.

11. In the manufacture of sheet glass, the steps consisting of drawing a sheet vertically from a bath of molten glass, acting upon the outer portions of the rising sheet with edge rollers while leaving its intermediate portion free, deflecting the sheet into another path at an angle to the vertical and horizontal after it passes the edge rollers, and passing it over a roller engaging the intermediate portion of the sheet.

12. In the manufacture of sheet glass, the steps consisting of drawing a sheet vertically from a glass bath, engaging it by opposed rolling surfaces while traveling vertically, and then deflecting it into a path at an angle to both the vertical and the horizontal.

13. In glass-making apparatus, means for drawing a plurality of separate and disconnected flat glass layers upwardly from molten glass, roller means for deflecting one of said layers independently of the other into another path, and means for bringing the two layers into contact and carrying them horizontally in a continuous manner.

14. In glass-making apparatus, means for drawing a plurality of separate and disconnected flat glass layers upwardly from molten glass, roller means for deflecting one of said layers independently of the other into another path, and roller means arranged to bend the other glass layer in a horizontal direction to bring the two layers into contact in a horizontal path.

15. In apparatus for making wire glass, means for drawing a plurality of separate

- and disconnected glass layers upwardly from molten glass, means for deflecting one of said layers independently of the other into another path, and roller means arranged to thereafter unite a plurality of layers with wire mesh between them and carry the wire glass in a horizontal direction.
16. In the manufacture of sheet glass, the steps consisting of drawing a sheet vertically from a glass bath, engaging it by opposed rolling surfaces while traveling vertically, then deflecting it into a path at an angle to both the vertical and the horizontal, and passing it over another deflecting roll which acts to flatten the sheet.
17. In the method of making wire glass, the steps consisting of continuously feeding molten glass to a heated receptacle wherein the glass rests as a liquid bath, continuously withdrawing from said receptacle two spaced apart ribbons of glass while maintaining the width thereof, bringing the ribbons together at a point spaced apart from the receptacle, and supplying wire mesh between the ribbons from a source lying within the space defined by the receptacle and the ribbons extending therefrom.
18. In the method of making wire glass, the steps consisting of continuously feeding molten glass to a heated receptacle wherein the glass rests as a liquid bath, continuously withdrawing from said receptacle two spaced apart ribbons of glass while maintaining the width thereof, bringing the ribbons together at a point spaced apart from the receptacle, and supplying wire mesh between the ribbons from a source lying within the space defined by the receptacle and the ribbons extending therefrom, the wire fabric being supplied to the glass adjacent the point where the glass ribbons are brought together.
19. In the method of making wire glass, the steps consisting of continuously feeding molten glass to a heated receptacle wherein the glass rests as a liquid bath, continuously withdrawing from said receptacle two spaced apart ribbons of glass while maintain-
- ing the width thereof, bringing the ribbons together at a point spaced apart from the receptacle, supplying wire mesh between the ribbons from a source lying within the space defined by the receptacle and the ribbons extending therefrom, the wire fabric being supplied to the glass adjacent the point where the glass ribbons are brought together, and pressing together the ribbons with the wire fabric therebetween.
20. In apparatus for making wire glass, a receptacle for molten glass, means for continuously feeding glass thereto, means for forming two spaced ribbons of glass from the bath in the receptacle and maintaining the width thereof, and a source of wire mesh fabric lying within the space defined by the receptacle and the ribbons extending therefrom to the point of union.
21. In apparatus for making wire glass, a receptacle for molten glass, means for continuously feeding glass thereto, means for forming two spaced ribbons of glass from the bath in the receptacle and maintaining the width thereof, a source of wire mesh fabric lying within the space defined by the receptacle and the ribbons extending therefrom to the point of union, and means for pressing the ribbons together with the wire mesh between them.
22. In the method of making wire glass, the steps consisting of continuously feeding molten glass from a tank furnace to a heated receptacle wherein the glass rests as a liquid bath, maintaining the same level in the receptacle as that of the tank furnace, continuously withdrawing from said heated receptacle two spaced apart ribbons of glass while maintaining their width, bringing the ribbons together at a point spaced apart from the receptacle, and supplying wire mesh between the ribbons from a source of mesh lying within the space defined by the heated receptacle and the ribbons extending therefrom.

In testimony whereof I have hereunto set my hand.

CLARENCE P. BYRNES.